

# United States Patent Office

2,739,869

Patented Mar. 27, 1956

1

2,739,869

## REMOVING DEPOSITS FROM DIAPHRAGMS EMPLOYED IN MANGANESE ELECTROWINNING

William A. Parsons, Knoxville, Tenn., assignor to Electro-Manganese Corporation, Knoxville, Tenn., a corporation of Delaware

No Drawing. Application July 19, 1952,  
Serial No. 299,916

3 Claims. (Cl. 8—137)

This invention relates to the art of electrowinning manganese from manganese sulfate-ammonium sulfate electrolytes. In that art direct electric current is passed through a manganese sulfate-ammonium sulfate electrolyte from anodes to cathodes and metallic manganese is deposited on the cathodes.

As is known, it is necessary to separate the electrolyte into two portions, catholyte and anolyte, since alkaline conditions are necessary for the deposition of manganese in the catholyte as distinguished from the acid conditions in the anolyte. Thus a typical pH range for the catholyte is from about 8.0 to 8.6 and for the anolyte from about 0.9 to 1.2, the former containing ammonium hydroxide and the latter sulfuric acid. To accomplish the required separation diaphragms are employed. Cotton canvas or duck has commonly been employed as diaphragm fabric. The maximum effective life of this material, e. g. 6-8 weeks, is so short that the cost of replacement is unduly high and the present invention is directed to improvements which make possible a diaphragm life of as much as two years with consequent very substantial savings.

The diaphragm assemblies differ somewhat, depending on the type of cell employed. In one type the cathodes are stainless steel sheets about 18" x 36" suspended in a diaphragm assembly or chamber having sides, ends, bottom and an open top. In the prior art this was essentially a cotton canvas or duck bag with a rectangular wood frame positioned therein to maintain the parts in spaced relation to the cathode with the sides lying in planes substantially parallel to the cathode. The anodes are bars or rods spaced from the diaphragm assemblies. In another type of cell the relation of anodes and cathodes to the diaphragm assemblies or chambers is reversed, that is, the anodes are positioned in the diaphragm chambers. In that type of cell the diaphragm assemblies or chambers are similar to those above mentioned except that they are open at the top and bottom, the bottom opening into a horizontal chamber partly defined by a false bottom parallel to and in spaced relation to the bottom of the cell. The anolyte is contained within the vertical diaphragm chambers or assemblies and the remainder of the cell above the false bottom then constitutes the catholyte chamber.

As is known, the electrowinning process is continuous, that is, the cell is continuously fed with purified catholyte and spent anolyte is continuously withdrawn and employed to extract manganese in the form of manganese sulfate from suitably conditioned ore and the extract after purification is fed back to the cell as catholyte. As the process proceeds continuously insoluble deposits are built up in and on the "anode side" surfaces of the diaphragm fabric, that is, the surfaces of the diaphragm fabric facing an anode in normal cell operation, and this phenomenon has created an obstacle to providing suitable diaphragms having a greatly improved life in relation to cotton canvas or duck. Indeed it is in the case of the more durable fabrics that the problem arises.

2

Thus, Jacobs et al., in Metal Industry, December 8, 1944, page 359, say:

"Wool, glass, Vinyon and micropore rubber backed with Vinyon were tested in the pilot plant. All of these materials are acid resistant but since they also must be discarded after 6 weeks because of the deposited calcium sulfate they have no advantage over canvas.

The limited teaching of the prior art in respect of the diaphragm fabric and the effective life thereof is also shown by the following quotation from "Electrolytic Manganese and its Alloys," by Reginald S. Dean, New York, The Ronald Press Company, 1952, page 54:

*Diaphragms.*—Canvas diaphragms have proved the most effective and economical. The diaphragms at Boulder City were 18-ounce non-waterproofed canvas. The voltage drop in the diaphragms increases with use, due to the deposition of calcium sulphate and reaches 0.2 volt in six weeks, at which time  $\frac{1}{4}$  inch of calcium sulphate will have accumulated on the diaphragm. At this point the diaphragm is discarded."

In accordance with the present invention diaphragm fabric made of polyacrylonitrile yarn is employed and by cleaning the said fabric at regular intervals by the method of the present invention, the life of the diaphragms is extended to as much as two years with consequent very substantial economic and other improvements. That diaphragm fabric has the following specific and preferred structure: It is a woven fabric composed of warp strands and filling strands consisting essentially of polyacrylonitrile yarn having 75 warp strands and 23 filling strands per linear inch, said strands being multiply 80 filament 200 denier yarns, the warp strands being 5-ply and the filling strands being 10-ply, the said fabric having a weight of about 18.5 ounces per square yard. Fabric having the stated physical and chemical characteristics possesses not only the physical characteristics necessary for successful functioning as diaphragm material in the cell but also the stability necessary to maintain those characteristics throughout repeated use periods in the cell and throughout repeated cleaning treatments as herein described.

The prior art has failed:

1. To appreciate the importance of cleaning the diaphragms at regular intervals and extending the life thereof.
2. To discover that not only calcium sulfate but also manganese dioxide causes plugging of the diaphragms by the deposits previously mentioned.
3. To provide an adequate method of cleaning which removes not only calcium sulphate but also manganese dioxide.

The invention will be defined in the claims and illustrated by the following specific example:

The diaphragm assembly or chamber, that is, the diaphragm fabric and its supporting frame, is removed from the electrolytic cell and soaked in a dilute solution of sulfuric acid containing from 2 to 10% preferably from 5 to 10% by weight of sulfuric acid, to dissolve manganese salts, loose metal, etc. The soaking time depends upon the amount of precipitated salts to be dissolved and is usually from 4 to 24 hours.

The second step is a treatment to remove calcium sulfate deposits from those surfaces of the diaphragm fabric which in cell operation face an anode. If the diaphragm assembly or chamber is one of the type within which a cathode is positioned during cell operation, the said assembly or chamber being open at the top and closed at the bottom, the said calcium sulfate insoluble deposits will form on the outside or "anode side" surfaces of the diaphragm fabric, since it is those surfaces which in cell operation face an anode. In that case the diaphragm assembly or chamber is placed in an upright position over a drain pan. It is filled with water and is maintained in

the filled condition by the delivery of water thereto. The solvent action of the water which passes through the fabric destroys the bond which holds the insoluble calcium sulfate deposits on the outside or opposite (the anode side) surfaces of the fabric, i. e. the surfaces which face an anode in normal cell operation, and those deposits either drop off or may easily be scraped from those surfaces. In this second step the time of treatment also varies from about 4 to 24 hours. If the diaphragm assembly or chamber is of the type within which an anode is positioned during cell operation, that is, open at the bottom as well as the top, then the insoluble calcium sulfate deposits are on the inside (anode side) of the diaphragm fabric, i. e. the fabric surfaces facing an anode in normal cell operation, and the procedure of the second step of the cleaning method is modified as follows: The diaphragm assembly after removing from the cell is mounted in a tank which may be a "dummy cell," that is, a tank similar to the electrolytic cell except for the absence of anodes, cathodes and electrolyte, water being used instead of the catholyte. A flow of water into and out of the said tank or "dummy cell" is preferably maintained because of the low solubility of calcium sulfate in water. In either case the principle of the second step of the cleaning method for removing difficultly soluble calcium sulfate deposits is the same, that is, a head of fresh water is maintained on the clean surfaces of the diaphragm fabric, that is, the surfaces facing a cathode in cell operation, and the combined solvent and pressure effects of the water which passes through the diaphragm fabric, loosen the calcium sulfate deposits so that they may be readily removed.

The third step is employed to dissolve manganese dioxide impregnated in the pores of the diaphragm fabric which the water does not remove in the second step. For that purpose the diaphragm assemblies or chambers are soaked in an aqueous  $MnO_2$  solvent, preferably a solution of sulfur dioxide containing from about 0.2 to 5 gs. per liter of sulfur dioxide and, preferably, from about 0.5 to 5% by weight of sulfuric acid. The use of sulfuric acid in addition to sulfur dioxide in the solution of the third step is not mandatory but is preferred because the solvent action of the sulfur dioxide is facilitated by the presence of sulfuric acid. The solution may also contain from 5 to 20% of ammonium sulfate.

Following the third step the diaphragm fabric is preferably rinsed or washed with water and the diaphragm assembly is returned to the cell.

The frequency of the above described cleaning method varies, depending upon the rate at which the insoluble deposits of manganese dioxide and calcium sulfate are formed. However, the periodic use of the method at intervals of 8 to 10 weeks has been found satisfactory in plant operation and when applied to the diaphragm fabrics made from polyacrylonitrile yarn has resulted in obtaining an effective life of those diaphragm fabrics of as much as two years, contra to the belief and teachings of the prior art.

While the invention has been described in terms of application to diaphragms made from polyacrylonitrile yarn, the cleaning method and its periodic use in obtaining a long effective life of the diaphragm are also applicable to diaphragms made from synthetic polymeric yarns when the diaphragm fabrics have physical structure and chemical properties (including resistance to attack by the electrolyte) substantially the same and equivalent to the diaphragm fabric specifically described herein.

While the above 3-step method is preferred, the said steps may be varied as follows: In the first step instead of sulfuric acid, an aqueous solution containing from 5 to 20% by weight of hydrochloric or nitric acid can be used.

In the second step, instead of water, a solution containing about 5 to 20% by weight of nitric, sulfuric or

hydrochloric acid may be used, or a solution containing 10 to 30% by weight of ammonium sulfate.

In the third step, instead of sulfur dioxide, or sulfur dioxide plus sulfuric acid or sulfur dioxide plus sulfuric acid and ammonium sulfate, other aqueous solvents for manganese dioxide may be used, e. g. a solution containing 5 to 10% by weight of ferrous sulfate and 5 to 10% by weight of sulfuric acid or a solution containing 5 to 10% by weight of hydrogen peroxide and 5 to 10% by weight of sulfuric acid or a solution containing 5 to 10% by weight of oxalic acid and 5 to 10% by weight of sulfuric acid, or a solution containing 5 to 20% by weight of hydrochloric acid. All of those reagents have a reducing effect on  $MnO_2$  which facilitates solution thereof.

Furthermore, all three steps may be combined into one step in a manner illustrated by the following method: The diaphragm assembly is removed from the cell, supported in an upright position and there is maintained on the clean surfaces of the diaphragm fabric, i. e. the surfaces facing a cathode in cell operation, a hydraulic head of an aqueous solution containing one of the following manganese dioxide solvents which also functions to loosen the calcium sulfate deposits, for a period of 4 to 24 hours until the calcium sulfate deposits on the opposite (anode) surfaces of the diaphragm fabric, i. e. the surfaces which face an anode in normal cell operation, are loosened and until the manganese dioxide impregnated in the pores of said diaphragm fabric are dissolved.

1. An aqueous solution containing from 0.2 to 5 gs. 30 per liter of  $SO_2$ , to which may be added from .5 to 5% by weight of sulfuric acid and 5 to 20% by weight of ammonium sulfate.

2. An aqueous solution containing from 5 to 10% by weight of ferrous sulfate and 5 to 10% by weight of  $H_2SO_4$ .

3. An aqueous solution containing from 5 to 10% by weight of  $H_2O_2$  and 5 to 10% by weight of  $H_2SO_4$ .

4. An aqueous solution containing 5 to 20% by weight of HCl.

40 The temperatures at which the herein described treatments are carried out are not critical. A range of temperatures from 25° C. to 40° C. is preferred although temperatures below 25° C. and above 40° C. may be employed, e. g. from about 10° C. to 80° C.

45 While it is preferred to remove the diaphragm assembly from the cell for cleaning said assembly, it is possible but not as convenient, to carry out the cleaning methods within the cell. For that purpose it is necessary to short circuit the cell, drain the electrolytes, i.e. catholyte and anolyte therefrom, and to use the cell essentially as a tank or container for holding or applying the cleaning reagents.

What is claimed is:

1. In the art of electrowinning manganese using an electrolytic cell containing a manganese sulfate-ammonium sulfate electrolyte and a diaphragm assembly comprising fabric made from polyacrylonitrile yarn supported on a framework to separate the electrolyte into catholyte and anolyte portions, and in which deposits of manganese dioxide and calcium sulfate form on and in the interstices of said fabric during normal use of the diaphragm assembly, the method of cleaning said diaphragm which comprises first removing the diaphragm assembly from the cell, immersing said assembly in a dilute sulfuric acid solution containing from about 2 to 10% by weight of sulfuric acid, for a period of about 4 to 24 hours; second, removing said assembly from said acid solution, supporting it in an upright position and maintaining the surfaces of the diaphragm fabric which face a cathode in cell operation in contact with water under a greater hydraulic head than acts on the opposite surfaces of said fabric until the calcium sulfate deposits formed on said opposite surfaces are loosened; third, immersing said diaphragm assembly in an aqueous solution of sulfur dioxide containing from about 0.2 to 5 gs.

per liter of sulfur dioxide and continuing said immersion for a period of about 4 to 24 hours to dissolve manganese dioxide impregnated in the pores of the diaphragm fabric, and, finally, washing said fabric with water.

2. In the art of electrowinning manganese using an electrolytic cell containing a manganous sulfate-ammonium sulfate electrolyte and a diaphragm assembly comprising fabric made from polyacrylonitrile yarn supported on a framework to separate the electrolyte into catholyte and anolyte portions, and in which deposits of manganese dioxide and calcium sulfate form on and in the interstices of said fabric during normal use of the diaphragm assembly, the method of cleaning said diaphragm fabric to restore the effectiveness of said diaphragm fabric for repeated use in the cell, which comprises, first removing the diaphragm assembly from the cell, immersing said assembly in a dilute acid solution containing from about 2 to 10% by weight of an acid of the group consisting of sulfuric acid, nitric acid, and hydrochloric acid for a period of about 4 to 24 hours; second, removing said assembly from said acid solution, supporting it in an upright position and maintaining the surfaces of the diaphragm fabric which face a cathode in normal cell operation in contact with a calcium sulfate dissolving reagent of the group consisting of water, an aqueous acid solution containing 5 to 10% by weight of sulfuric acid, an aqueous acid solution containing about 5 to 10% by weight of hydrochloric acid, and an aqueous solution containing about 5 to 10% by weight of nitric acid, said aqueous reagent being maintained under a greater hydraulic head than acts on the opposite surfaces of said fabric, until the calcium sulfate deposits on said opposite surfaces are loosened, and removing said deposits; third, immersing said diaphragm assembly in an aqueous manganese dioxide solvent of the group consisting of an aqueous solution containing from about 0.2 to 5 gs. per liter of sulfur dioxide, an aqueous solution containing from 5 to 10% by weight of ferrous sulfate and 5 to 10% sulfuric acid, an aqueous solution containing from 5 to 10% by weight of hydrogen peroxide and 5 to 10% by weight of sulfuric acid, an aqueous solution containing from 5 to 10% by weight of oxalic acid and 5 to 10% by weight of sulfuric acid, and an

5

aqueous solution containing 5 to 20% by weight of hydrochloric acid, and continuing said immersion for a period of about 4 to 24 hours to dissolve manganese dioxide impregnated in the pores of said diaphragm fabric.

10

3. In the art of electrowinning manganese using an electrolytic cell containing a manganous sulfate-ammonium sulfate electrolyte and a diaphragm assembly comprising fabric made from polyacrylonitrile yarn supported on a framework to separate the electrolyte into catholyte and anolyte, and in which deposits of manganese dioxide and calcium sulfate form on and in the interstices of said fabric during normal use of the diaphragm assembly, the method of cleaning said diaphragm fabric to restore the effectiveness of said diaphragm fabric for repeated use in the cell, which comprises removing said diaphragm assembly from the cell, supporting it in an upright position and maintaining the surfaces of the diaphragm fabric facing a cathode in normal cell operation in contact with a manganese dioxide dissolving reagent of the group consisting of an aqueous solution containing from 0.2 to 5 gs. per liter of sulfur dioxide, an aqueous solution containing from 5 to 10% by weight of ferrous sulfate and from 5 to 10% by weight of sulfuric acid, an aqueous solution containing from 5 to 10% by weight of hydrogen peroxide and 5 to 10% by weight sulfuric acid, and an aqueous solution containing 5 to 20% by weight of hydrochloric acid, until the calcium sulfate deposits on the opposite surfaces of the diaphragm fabric are loosened and until the manganese dioxide impregnated in the pores of said diaphragm fabric is dissolved.

#### References Cited in the file of this patent

#### UNITED STATES PATENTS

|           |                 |              |
|-----------|-----------------|--------------|
| 442,335   | Roberts -----   | Dec. 9, 1890 |
| 1,120,629 | Salisbury ----- | Dec. 8, 1914 |

#### FOREIGN PATENTS

|         |              |               |
|---------|--------------|---------------|
| 460,564 | Canada ----- | Oct. 25, 1949 |
|---------|--------------|---------------|

#### OTHER REFERENCES

Jacobs et al.: Metal Industry, December 8, 1944, p. 359.